

March 11, 1930.

J. C. McFARLAND

1,750,418

ETCHING AND DECORATING METAL SURFACES

Filed Dec. 5, 1928

Fig. 1.



Fig. 2.



Fig. 3.



Fig. 4.



Fig. 5.



Fig. 6.



Fig. 7.



Fig. 8.



Inventor:

James C. McFarland,  
By J. Grenforth Lee, Christopher Miles,  
Attny.

Patented Mar. 11, 1930

1,750,418

# UNITED STATES PATENT OFFICE

JAMES C. MCFARLAND, OF FORT THOMAS, KENTUCKY, ASSIGNOR TO THE WADSWORTH WATCH CASE CO., OF DAYTON, KENTUCKY, A CORPORATION OF KENTUCKY

## ETCHING AND DECORATING METAL SURFACES

Application filed December 5, 1928. Serial No. 324,024.

This invention relates particularly to a method of decorating and/or etching metal surfaces. The invention relates more especially to a method of decorating base metal surfaces as by plating and/or etching.

The primary object is to provide a simple and effective method which is well adapted for use in decorating the surfaces of base metals, such as steel, 12% nickel alloy, etc. 10 A nickel alloy of the character just referred to and which is in common use is composed of Ni, 12%; Cu, 70%; Zn, 18%.

The invention will be described first with reference to the treatment of a steel plate, or block, by way of example. Such method 15 is illustrated in the accompanying drawing, in which—

Fig. 1 represents a base plate, which may be of steel; Fig. 2 is intended to illustrate the 20 application of a copper plating to the base plate; Fig. 3 illustrates a further step in which a suitable resist design is applied to the copper plating; Fig. 4 represents a further 25 step in which the exposed areas of copper are removed, as by means of a suitable solvent for copper; Fig. 5 illustrates a further step in which the resist design has been removed, leaving areas of the original metal exposed and other areas covered with the 30 copper plating; Fig. 6 illustrates a further step in which a chromium plating is applied to the exposed areas of the steel plate, so that the plate now bears a design in copper plating and a complementary design in chromium plating; Fig. 7 illustrates a further 35 step in which the remaining copper plating is removed; and Fig. 8 represents a further step in which gold plating is applied to the newly exposed areas of the steel surface, so that the 40 steel plate now has a surface composed of a chromium plating design and a complementary gold plating design.

If desired, a further step may be used. That is, the remaining chromium plating may 45 be removed and the newly exposed surfaces of

the steel plate may be etched, whilst the gold plating serves as a resist. This step may be followed by a further step in which the etched areas of the steel plate are given a plating contrasting in color with the gold plating.

In applying a chromium plating as illustrated in Fig. 6, one uses a suitable current density (amperage per unit of area), which will result in the steel areas taking the chromium plating, while the copper areas will not receive the chromium plating. Methods enabling this to be accomplished are known in the art.

Referring to Fig. 8, the exposed steel surfaces will receive the gold plating, while the 60 chromium plating will not receive the gold plating.

If desired to remove the chromium plating shown in Fig. 8, a suitable solvent for the purpose is dilute hydrochloric acid, or dilute 65 sulphuric acid. Chromium plating is hard, resistant and free from tarnishing. It possesses a color somewhat similar to aluminum. It therefore affords a color which contrasts with the gold color and may be allowed to 70 remain as a part of the decorative design, if desired.

Any precious metal, or precious metal alloy, may be used in lieu of gold. Where complementary designs of different metals are desired in a complete decorative design, one selects metals of contrasting colors.

Ferric chloride may be used for etching the base plate. Any other suitable plating may be used in lieu of copper plating, as, for example, brass plating.

Brasses, bronzes, German silvers, etc. may, by suitable variations in the process, be used as base plates. One may, in the first instance, provide a base plate with complementary 85 designs in different metals, and may then proceed to apply a chromium plating to one of the metals, by using suitable conditions for effecting the deposit of the chromium plating upon one of the metals and not on the other.

The chromium plating may then serve as a resist while a precious metal plating is being applied to the areas not covered by the chromium plating. Finally, the chromium plating may be removed, or not, as desired; and if removed, the newly exposed metal may be etched, and the etching operation may be followed by a further plating operation, if desired.

10 The resist design may be applied in any suitable manner, as by a transfer method, or by a photographic method. In the example given above, the resist design preferably is produced by applying to the copper plating a light-sensitive varnish; photographically producing an image in the varnish; and finally subjecting the film to a developing operation which dissolves the unreacted portions of the varnish, thus leaving a suitable resist 15 design upon the copper plate.

Where the base plate is of steel, nitric acid may be used for etching the plate. Any suitable etching agent may be used, depending upon the metal of which the base plate is 20 composed.

The foregoing detailed description has been given for clearness of understanding only, and no unnecessary limitations should be understood therefrom, but the appended claims 30 should be construed as broadly as permissible, in view of the prior art.

What I regard as new, and desire to secure by Letters Patent, is:

1. The method of treating a metal surface, 35 which comprises: producing complementary designs in different metals; and subjecting the surface to an electroplating operation with chromium at such current density as to cause the chromium plating to be applied to 40 one design and not to the other.

2. The method of treating a base metal surface, which comprises: applying a metal plating to the surface; applying a resist design to said plating; removing said plating 45 at the exposed areas; and electroplating with chromium the areas of one metal by employing a current density which will cause the deposition of the chromium upon such metal without plating the other metal.

50 3. The method of treating a base metal surface, which comprises: plating the surface; applying a suitable resist design to said plating; dissolving said plating at the unprotected areas; removing said resist design; 55 electroplating with chromium the areas presented by one of the metals, using such current density that the other areas will not be plated; removing by means of a suitable solvent the remainder of the first-mentioned 60 plating; and plating with precious metal the last exposed areas.

4. The method of treating a base metal surface, which comprises: plating the surface; applying a suitable resist design to said 65 plating; dissolving said plating at the un-

protected areas; removing said resist design; electroplating with chromium the areas presented by one of the metals, using such current density that the other areas will not be plated; removing by means of a suitable solvent 70 the remainder of the first-mentioned plating; plating with precious metal the last exposed areas; removing the chromium plating; and etching the surface exposed by the removal of the chromium plating.

JAMES C. McFARLAND.

75

80

85

90

95

100

105

110

115

120

125

130